

1

2,943,935

## STABILIZATION OF PHOTOGRAPHIC BLEACH POWDERS CONTAINING AN ALKALI METAL FERRICYANIDE

Lawrence G. Welliver, Binghamton, N.Y., assignor to General Aniline &amp; Film Corporation, New York, N.Y., a corporation of Delaware

No Drawing. Filed May 15, 1957, Ser. No. 659,213

10 Claims. (Cl. 96—60)

The present invention relates to single powder photographic bleach mixtures containing an alkali metal ferricyanide as the oxidizing agent, and more particularly to the stabilization of such bleach powders.

Most photographic bleach solutions which are used for the processing of color film contain in aqueous solution an alkali metal ferricyanide such as lithium, potassium or sodium ferricyanide as the oxidizing agent which converts the metallic silver formed during development into a silver salt which is soluble in silver halide solvents such as hypo. Typically, such a bleach solution contains, in addition to the ferricyanide, a halogenizing or converting agent preferably an alkali metal chloride or an alkali metal bromide which converts the silver ferricyanide initially formed in the bleaching reaction into the less soluble silver chloride or silver bromide and thus impels the bleach reaction to completion.

It is essential that the bleach reaction be carried out at a pre-selected pH and consequently, the ferricyanide bleach solutions contain a buffering agent which maintains the desired pH even though small amounts of acids or alkali may be carried into the bleach by the film. The pH of the bleach solutions falls between a range of from 3 to 9, a pH between 4 and 6 being generally preferred. Among the more frequently used ingredients of such buffer mixtures are alkali metal phosphates such as disodium and monosodium phosphate, sodium citrate, sodium bisulfate, citric acid or phthalic acid. Some of the ingredients of the buffer mixture act also as corrosion inhibitors and retard the corrosive action of the ferricyanide bleach on metallic developing tanks, trays and the like.

For reasons of economy and convenience, the alkali metal ferricyanide bleaches are usually packaged and sold as dry powder mixtures. Normally, the stability of dry ferricyanide bleach mixtures leaves much to be desired. However, their stability is further drastically curtailed by the presence of other ingredients which are added to ensure that the bleach possesses certain desirable photographic characteristics.

For instance, a metal ferrocyanide is included which gives a tempering action to a freshly mixed bleach solution in order to simulate the performance of a partially used bleach. The rate of bleaching depends on the oxidation reduction potential which in turn is a function of pH and the relative ferrocyanide-ferricyanide concentration. No such oxidation reduction potential can be established so long as ferricyanide only is in the fresh solution, and no ferrocyanide has been formed as a result of the bleaching action. The desired tempering action is achieved by adding to a fresh bleach solution specified amounts of ferrocyanide thus establishing an oxidation reduction potential which otherwise would be set up only after part of the ferricyanide had been reduced to ferrocyanide.

In such powder admixtures, the ferricyanide has an even greater tendency to cause caking and discoloration. It is believed that this discoloration is caused by the de-

2

composition of ferricyanide yielding ferrocyanide and iron salts leading in all likelihood to the formation of Prussian Blue or Turnbull's Blue. As a by-product, a gas is formed which creates a pressure build-up in hermetically sealed packages. This gas has been identified as hydrogen cyanide which is highly toxic. Thus, the decomposition of ferricyanide bleach powders creates a serious health hazard. Other ingredients which affect adversely the stability of the ferricyanide bleaching powder are alkali dichromates which are added to bleach solutions to inhibit the corrosion of processing equipment. Ferricyanide bleaches containing dichromates also cake and discolor with the formation of hydrogen cyanide.

I have discovered that boric anhydride is an effective stabilizer for photographic bleaches particularly those which contain, in addition to the alkali metal ferricyanide, a small amount of alkali ferrocyanide or alkali dichromate. Photographic bleach mixtures containing alkali metal ferricyanide as the oxidizing agent and stabilized with boric anhydride constitute the purposes and objects of the present invention.

The photographic bleach powders which are contemplated herein contain as their essential ingredients an alkali metal ferricyanide and boric anhydride, together with other bleach adjuvants including buffer mixtures, alkali metal halides, particularly alkali metal bromides and alkali metal ferrocyanides or alkali metal dichromates. Photographic bleach powders which we have found stable during storage for considerable periods of time may be compounded in the following proportions, it being understood that all parts are by weight and that the resulting dry powder is to be used to make a liter of bleach solution:

|                              | Parts     |
|------------------------------|-----------|
| 35 Alkali metal ferricyanide | 30 to 120 |
| Alkali metal halide          | 2 to 20   |
| Buffer mixture               | 5 to 30   |
| Alkali metal ferrocyanide    | 2 to 12   |
| or                           |           |
| 40 Alkali metal dichromate   | 2 to 12   |
| Boric anhydride              | 4 to 25   |

In compounding the above bleach powder, one may proceed by mixing the boric anhydride to the alkali metal ferricyanide and adding the other ingredients later. However, if preferred, all the ingredients may be admixed simultaneously. One of the most important advantages of boric anhydride lies in the fact that its stabilizing action is not impaired by changes in alkalinity and acidity.

50 In spite of the anhydrous nature of the boric anhydride, it is surprising to note that the stabilizing action is not based on a dehydrating action and is not influenced by the selection of bleach ingredients with different amounts of water of crystallization.

55 While it is desirable to use a grade of boric anhydride which is completely free of water, it must be kept in mind that small amounts of moisture are absorbed by the anhydride during storage and before the mixing of the bleach. However, these small amounts of water absorbed which usually do not exceed 2 percent, but which may go up as high as 5 percent based on the weight of boric anhydride, do not interfere with the stabilizing action on the bleach powder.

60 The following examples will serve to illustrate my invention but are not restricted thereto. The quantity of the bleach mixtures represented by the following formulae is to be dissolved in sufficient water to give one liter of bleach solution.

## Example I

|                           | Grams |
|---------------------------|-------|
| 70 Potassium ferricyanide | 50.0  |
| Potassium ferrocyanide    | 5.0   |

|                    |      |
|--------------------|------|
| Sodium bromide     | 15.0 |
| Disodium phosphate | 11.0 |
| Citric acid        | 8.0  |
| Boric anhydride    | 10.0 |

This powder mixture, which contained potassium ferricyanide, did not deteriorate after incubation at 120° F. for 72 hours or storage for 3 months at room temperature (72° F.). Under the same testing conditions, an identical powder mixture from which the boric anhydride was omitted, was badly caked and discolored to a deep blue color with the formation of highly toxic hydrogen cyanide gas.

*Example II*

|                        |       |
|------------------------|-------|
|                        | Grams |
| Potassium ferricyanide | 50.0  |
| Potassium ferrocyanide | 5.0   |
| Sodium bromide         | 15.0  |
| Monosodium phosphate   | 10.0  |
| Phthalic acid          | 2.0   |
| Boric anhydride        | 10.0  |

This powder mixture did not deteriorate during incubation for one week at 110° F. or after storage at room temperature for 6 months. By comparison, a similar powder mixture from which the boric anhydride was omitted, was badly caked and discolored to a light blue color with the formation of highly toxic hydrogen cyanide gas.

*Example III*

|                        |       |
|------------------------|-------|
|                        | Grams |
| Potassium ferricyanide | 50.0  |
| Potassium dichromate   | 5.0   |
| Sodium bromide         | 15.0  |
| Citric acid            | 2.0   |
| Boric anhydride        | 10.0  |

This powder mixture which contained potassium dichromate did not deteriorate during incubation for one week at 120° F. or storage at room temperature (74° F.) for six months. A comparison mixture from which the boric anhydride had been omitted was submitted to the same storage conditions. It caked and discolored to a deep blue color with the formation of highly toxic hydrogen cyanide gas.

*Example IV*

|                        |       |
|------------------------|-------|
|                        | Grams |
| Potassium ferricyanide | 100.0 |
| Potassium ferrocyanide | 7.5   |
| Sodium bromide         | 20.0  |
| Disodium phosphate     | 12.0  |
| Citric acid            | 9.0   |
| Boric anhydride        | 15.0  |

This powder mixture did not deteriorate after storage for 6 months at an average room temperature of 75° F. An identical powder mixture from which the boric anhydride was omitted was badly caked and discolored to a deep blue color after a few days.

*Example V*

|                        |       |
|------------------------|-------|
|                        | Grams |
| Potassium ferricyanide | 30.0  |
| Potassium dichromate   | 3.0   |
| Sodium bromide         | 10.0  |
| Citric acid            | 2.0   |
| Boric anhydride        | 5.0   |

This powder mixture was kept for 6 months at room temperature without deterioration. A mixture without boric anhydride caked badly after a few days and discolored to a deep blue color with the formation of hydrogen cyanide gas.

*Example VI*

|                        |       |
|------------------------|-------|
|                        | Grams |
| Potassium ferricyanide | 75.0  |
| Potassium ferrocyanide | 5.0   |
| Sodium bromide         | 10.0  |

|                      |      |
|----------------------|------|
| Monosodium phosphate | 10.0 |
| Phthalic acid        | 4.0  |
| Boric anhydride      | 12.0 |

This powder mixture did not deteriorate when stored for 6 months at room temperature. A type mixture from which the boric anhydride had been omitted became discolored and caked badly after a few days.

Various modifications such as substituting equivalent materials and varying the proportions of materials used will be obvious to persons skilled in the art. Therefore, the scope of the invention is to be limited solely by the appended claims.

I claim:

1. A stable single powder photographic bleach mixture containing as its essential components from 30 to 120 parts by weight of an alkali metal ferricyanide, from 2 to 20 parts by weight of an alkali metal bromide, from 4 to 25 parts of boric anhydride and from 2 to 12 parts by weight of an alkali metal ferrocyanide, the parts being based on the total weight of the powder.

2. A stable single powder photographic bleach mixture containing as its essential components from 30 to 120 parts by weight of an alkali metal ferricyanide, from 2 to 20 parts by weight of an alkali metal bromide, from 4 to 25 parts of boric anhydride and from 2 to 12 parts by weight of an alkali metal dichromate, the parts being based on the total weight of the powder.

3. A stable single powder photographic bleach mixture containing as its essential ingredients for the preparation of one liter of bleach solution: from 30 to 120 parts by weight of alkali metal ferricyanide; from 2 to 20 parts by weight of alkali metal bromide; from 5 to 30 parts by weight of a buffer mixture comprising a salt selected from the group consisting of alkali metal phosphates and alkali metal citrates, and an acid selected from the group consisting of citric and phthalic acid; and from 4 to 25 parts by weight of boric anhydride, the parts being based on the total weight of the powder.

4. A stable single powder photographic bleach mixture containing as its essential ingredients for the preparation of one liter of bleach solution: from 30 to 120 parts by weight of alkali metal ferricyanide; from 2 to 20 parts by weight of alkali metal bromide; from 5 to 30 parts by weight of a buffer mixture comprising a salt selected from the group consisting of alkali metal phosphates and alkali metal citrates, and an acid selected from the group consisting of citric and phthalic acid; from 4 to 25 parts by weight of boric anhydride; and from 2 to 12 parts by weight of alkali metal ferrocyanide, the parts being based on the total weight of the powder.

5. A stable single powder photographic bleach mixture containing as its essential ingredients for the preparation of one liter of bleach solution: from 30 to 120 parts by weight of alkali metal ferricyanide; from 2 to 20 parts by weight of alkali metal bromide; from 5 to 30 parts by weight of a buffer mixture comprising a salt selected from the group consisting of alkali metal phosphates and alkali metal citrates, and an acid selected from the group consisting of citric and phthalic acid; from 4 to 25 parts by weight of boric anhydride; and from 2 to 12 parts by weight of alkali metal dichromate, the parts being based on the total weight of the powder.

6. A stable single powder photographic bleach mixture comprising an alkali metal ferricyanide, an alkali metal ferrocyanide, an alkali metal bromide and a stabilizing amount of boric anhydride in a quantity sufficient to prevent caking and discoloration of said bleach mixture.

7. A stable single powder photographic bleach mixture comprising an alkali metal ferricyanide, an alkali metal bromide, a buffer mixture comprising a member selected from the group consisting of alkali metal phosphates and alkali metal citrates and a member selected from the group of citric acid and phthalic acid, and a stabilizing amount of boric anhydride in a quantity sufficient to prevent caking and discoloration of said bleach mixture.

8. A stable photographic bleach mixture having the following composition:

|                        | Grams |
|------------------------|-------|
| Potassium ferricyanide | 50.0  |
| Potassium ferrocyanide | 5.0   |
| Sodium bromide         | 15.0  |
| Disodium phosphate     | 11.0  |
| Citric acid            | 8.0   |
| Boric anhydride        | 10.0  |

9. A stable photographic bleach mixture having the following composition:

|                        | Grams |
|------------------------|-------|
| Potassium ferricyanide | 50.0  |
| Potassium dichromate   | 5.0   |
| Sodium bromide         | 15.0  |
| Citric acid            | 2.0   |
| Boric anhydride        | 10.0  |

10. A stable photographic bleach mixture having the following composition:

|                        | Grams |
|------------------------|-------|
| Potassium ferricyanide | 50.0  |
| Potassium ferrocyanide | 5.0   |
| Sodium bromide         | 15.0  |
| Monosodium phosphate   | 10.0  |
| Phthalic acid          | 2.0   |
| Boric anhydride        | 10.0  |

10. References Cited in the file of this patent

UNITED STATES PATENTS

|              |                |
|--------------|----------------|
| Plagwitz     | Jan. 17, 1928  |
| Rogers       | Aug. 5, 1952   |
| Zappert      | Sept. 23, 1952 |
| Boyer et al. | Sept. 1, 1953  |
| Kridel       | July 15, 1958  |